



1

## TECHNICAL FIELD

The present invention relates to a yellow toner which provides a sharper color than ever before in small amounts and which has excellent light resistance.

## BACKGROUND ART

In an image forming device such as an electrophotographic device and an electrostatic recording device, first, an electrostatic latent image formed on the photoconductor is developed with a toner. Next, as needed, a toner image thus formed is transferred onto a transfer material such as a paper sheet and then fixed thereon by various methods such as heating, pressurization or solvent fume.

In the field of such an image forming device, a digital full-color copying machine and a digital full-color printer have been put to practical use. A digital full-color copying machine produces a full-color image as follows. First, an original color image is subjected to color separation with blue, green and red filters; an electrostatic latent image corresponding to the original color image, which is composed of dots that are 20 to 70  $\mu\text{m}$  in diameter, is developed with yellow, magenta, cyan and black toners; and a full-color image is formed using the subtractive color mixing effect.

Recently, there is an increasing demand for full-color images with high image quality and high resolution. Especially, to increase color reproducibility, it is hoped that an image can be printed in the same hue as ink printing.

As a color pigment for a yellow toner, for example, a disazo pigment as typified by C.I. Pigment Yellow 12, 13 and 17, and a monoazo pigment as typified by C.I. Pigment Yellow 74, 97 and 98 have been generally used.

Besides the combinations of yellow pigments, examples of improving toner properties by combining a yellow pigment and a yellow dye, are known.

Patent Literature 1 discloses a yellow toner comprising C.I. Pigment Yellow 74 and C.I. Solvent Yellow 162. In Patent Literature 1, it is described that by containing these colorants, the toner obtains satisfactory color tone that is obtained in the case of incorporating C.I. Pigment Yellow 74 solely in a toner, and high coloring power of C.I. Solvent Yellow 162.

Patent Literature 2 discloses a yellow toner comprising, as colorants, C.I. Pigment Yellow 155 and C.I. Solvent Yellow 162 at a specific ratio. Patent Literature 2 describes that due to the colorants contained at the specific ratio and due to the excellent compatibility of C.I. Solvent Yellow 162 with binder resin, the dispersibility of C.I. Pigment Yellow 155 can be further increased, and more stable charging property and better transparency can be obtained.

Patent Literature 3 discloses a yellow toner comprising C.I. Solvent Yellow 162, a condensed azo pigment (e.g., C.I. Pigment Yellow 93) and so on. Patent Literature 3 describes that the aggregation of the condensed azo pigment (e.g., C.I. Pigment Yellow 93) can be suppressed by the use of C.I. Solvent Yellow 162, so that the dispersibility of the condensed azo pigment can be increased, and more uniform triboelectric chargeability can be obtained.

## CITATION LIST

Patent Literature 1: Japanese Patent Application Laid-open (JP-A) No. 2006-126384

Patent Literature 2: JP-A No. 2006-313302

Patent Literature 3: JP-A No. 2000-162824

2

## SUMMARY OF INVENTION

## Technical Problem

5 The applications of an electrophotographic image forming device have been extended from general copying machines and printers used to print or copy office documents, to the field of production of printed matters for use outside the office, in particular, to the print-on-demand (POD) market that is an area of quick printing, since the image forming device can easily print variable information from electronic data. Therefore, in recent years, the level of demand required of the reflection density and chroma of a printed product has been rapidly increased.

Unlike a pigment, a dye is characterized by solubility in solvents and poor resistance to light. Accordingly, a combination of a dye and a pigment has a problem in that there is a decrease in light resistance when the content ratio of the dye is too large. Therefore, a limitation is imposed on the content ratio of the dye and the pigment.

From the viewpoint of downsized image forming devices and less energy consumption, there is a demand for reduction in toner consumption in printing. However, printing with a small amount of toner has a problem in that there is a decrease in chroma and color gamut. Also, the toners using the dyes described in Patent Literatures 1 to 3 cannot obtain a sufficiently wide color range when the toner amount is small.

30 An object of the present invention is to provide a yellow toner which provides a sharper color than ever before in small amounts and which has excellent light resistance.

### Solution to Problem

To attain the object, the inventor of the present invention conducted detailed research and found the following: by using the combination of compounds A and B as a yellow colorant, each of which has a specific chemical structure, a yellow toner which provides a sharper color than ever before in small amounts and which has excellent light resistance, is obtained. Based on this finding, the inventor achieved the present invention.

45 That is, the yellow toner of the present invention is a yellow toner comprising a binder resin and a yellow colorant, wherein a compound A represented by the following general formula (1) and a compound B represented by the following general formula (2) are contained as the yellow colorant, and wherein a total content of the compound A and the compound B is from 3 to 30 parts by mass with respect to 100 parts by mass of the binder resin, and a mass ratio of the content of the compound A to the content of the compound B (compound A/compound B) is from 0.8 to 20:

### General Formula (1)



65 where  $R^{1A}$ ,  $R^{1B}$ ,  $R^{2A}$  and  $R^{2B}$  are each independently a halogen atom, an alkyl group, a methoxy group, an amino

group, a nitro group, an acetyl amido group ( $-\text{NHCOCH}_3$ ), a methyl ester group ( $-\text{COOCH}_3$ ) or a primary amide group ( $-\text{CONH}_2$ );  $R^3$  is a halogen atom;  $R^4$  and  $R^5$  are each independently a halogen atom, an alkyl group, a methoxy group, an amino group, a nitro group, an acetyl amido group ( $-\text{NHCOCH}_3$ ), an acetyl group ( $-\text{COCH}_3$ ), a methyl ester group ( $-\text{COOCH}_3$ ) or a primary amide group ( $-\text{CONH}_2$ );  $a_1$  and  $b_1$  are positive integers that a sum of the positive integers is 1 or more and 3 or less;  $a_2$  and  $b_2$  are positive integers that a sum of the positive integers is 1 or more and 3 or less;  $c$  is an integer of 1 or more and 3 or less; and  $d$  and  $e$  are each independently 1 or 2.



General Formula (2) 15

where  $R^6$  is an alkyl group.

#### Advantageous Effects of Invention

According to the present invention as described above, by using the compound A having the chemical structure represented by the general formula (1) in combination with the compound B having the chemical structure represented by the general formula (2), the dispersion stability of the compounds in the polymerizable monomer composition or binder resin is increased; therefore, a yellow toner which provides a sharper color than ever before in small amounts and which has excellent light resistance, is provided.

#### DESCRIPTION OF EMBODIMENTS

The yellow toner of the present invention is a yellow toner comprising a binder resin and a yellow colorant, wherein a compound A represented by the following general formula (1) and a compound B represented by the following general formula (2) are contained as the yellow colorant, and wherein a total content of the compound A and the compound B is from 3 to 30 parts by mass with respect to 100 parts by mass of the binder resin, and a mass ratio of the content of the compound A to the content of the compound B (compound A/compound B) is from 0.8 to 20:

General Formula (1)



where  $R^{1A}$ ,  $R^{1B}$ ,  $R^{2A}$  and  $R^{2B}$  are each independently a halogen atom, an alkyl group, a methoxy group, an amino group, a nitro group, an acetyl amido group ( $-\text{NHCOCH}_3$ ), a methyl ester group ( $-\text{COOCH}_3$ ) or a primary amide group ( $-\text{CONH}_2$ );  $R^4$  and  $R^5$  are each

independently a halogen atom, an alkyl group, a methoxy group, an amino group, a nitro group, an acetyl amido group ( $-\text{NHCOCH}_3$ ), an acetyl group ( $-\text{COCH}_3$ ), a methyl ester group ( $-\text{COOCH}_3$ ) or a primary amide group ( $-\text{CONH}_2$ );  $a_1$  and  $b_1$  are positive integers that a sum of the positive integers is 1 or more and 3 or less;  $a_2$  and  $b_2$  are positive integers that a sum of the positive integers is 1 or more and 3 or less;  $c$  is an integer of 1 or more and 3 or less; and  $d$  and  $e$  are each independently 1 or 2.

General Formula (2)



where  $R^6$  is an alkyl group.

Hereinafter, the yellow toner of the present invention may be simply referred to as "toner".

Hereinafter, a method for producing yellow colored resin particles used in the present invention (hereinafter they may be simply referred to as "colored resin particles"), yellow colored resin particles obtained by the production method, a method for producing a yellow toner using the yellow colored resin particles, and the yellow toner of the present invention will be described in order.

#### 1. Method for Producing Colored Resin Particles

In general, methods for producing colored resin particles are broadly classified into dry methods such as a pulverization method and wet methods such as an emulsion polymerization agglomeration method, a suspension polymerization method and a solution suspension method. The wet methods are preferred since a toner that has excellent printing characteristics such as image reproducibility can be easily obtained. Among the wet methods, polymerization methods such as the emulsion polymerization agglomeration method and the suspension polymerization method are preferred, since a toner that has relatively small particle size distribution in micron order can be easily obtained. Among the polymerization methods, the suspension polymerization method is more preferred.

The emulsion polymerization agglomeration method is a method for producing colored resin particles by polymerizing emulsified polymerizable monomers to obtain a resin microparticle emulsion, and aggregating the resulting resin microparticles with a colorant dispersion, etc. The solution suspension method is a method for producing colored resin particles by forming droplets of a solution in an aqueous medium, the solution containing toner components such as a binder resin and a colorant dissolved or dispersed in an organic solvent, and removing the organic solvent. Both methods can be carried out by known methods.

The colored resin particles used in the present invention can be produced by the wet methods or the dry methods. The wet methods are preferred, and among the wet methods, the suspension polymerization method is particularly preferred. By the suspension polymerization method, the colored resin particles are produced through the processes described below.

## (A) Suspension Polymerization Method

## (A-1) Preparation Process of Polymerizable Monomer Composition

First, a polymerizable monomer, a yellow colorant, and other additives added as needed, such as a charge control agent and a release agent, are mixed to prepare a polymerizable monomer composition. For example, a media type dispersing machine is used for the mixing in the preparation of the polymerizable monomer composition.

In the present invention, the polymerizable monomer means a monomer having a polymerizable functional group, and the polymerizable monomer is polymerized into a binder resin. As a main component of the polymerizable monomer, a monovinyl monomer is preferably used. As the monovinyl monomer, examples include, but are not limited to, styrene; styrene derivatives such as vinyl toluene and  $\alpha$ -methylstyrene; acrylic acid and methacrylic acid; acrylic acid esters such as methyl acrylate, ethyl acrylate, propyl acrylate, butyl acrylate, 2-ethylhexyl acrylate and dimethylaminoethyl acrylate; methacrylic acid esters such as methyl methacrylate, ethyl methacrylate, propyl methacrylate, butyl methacrylate, 2-ethylhexyl methacrylate and dimethylaminoethyl methacrylate; nitrile compounds such as acrylonitrile and methacrylonitrile; amide compounds such as acrylamide and methacrylamide; and olefins such as ethylene, propylene and butylene. These monovinyl monomers may be used alone or in combination of two or more kinds. Among them, styrene, styrene derivatives, and derivatives of acrylic acids or methacrylic acids are preferably used as the monovinyl monomer.

In order to improve hot offset and storage stability, it is preferable to use a crosslinkable polymerizable monomer together with the monovinyl monomer. The crosslinkable polymerizable monomer means a monomer having two or more polymerizable functional groups. As the crosslinkable polymerizable monomer, examples include, but are not limited to, aromatic divinyl compounds such as divinyl benzene, divinyl naphthalene and derivatives thereof; ester compounds in which two or more carboxylic acids are esterified to alcohol having two or more hydroxyl groups, such as ethylene glycol dimethacrylate and diethylene glycol dimethacrylate; other divinyl compounds such as N,N-divinylaniline and divinyl ether; and compounds having three or more vinyl groups. These crosslinkable polymerizable monomers can be used alone or in combination of two or more kinds.

In the present invention, it is desirable that the amount of the crosslinkable polymerizable monomer is generally from 0.1 to 5 parts by mass, and preferably from 0.3 to 2 parts by mass, with respect to 100 parts by mass of the monovinyl monomer.

Also, it is preferable to use a macromonomer as a part of the polymerizable monomer, since the balance between the storage stability and low-temperature fixability of the toner to be obtained can be improved. The macromonomer is a reactive oligomer or polymer having a polymerizable carbon-carbon unsaturated double bond at the end of a polymer chain and generally having a number average molecular mass of from 1,000 to 30,000. The macromonomer is preferably one that can provide a polymer having a higher glass transition temperature (hereinafter may be referred to as "Tg") than a polymer obtained by polymerization of a monovinyl monomer. The amount of the macromonomer is preferably from 0.03 to 5 parts by mass, and more preferably from 0.05 to 1 part by mass, with respect to 100 parts by mass of the monovinyl monomer.

In the present invention, the compound A and the compound B are contained as the yellow colorant.

Hereinafter, the compound A used in the present invention will be described in detail.

The compound A of the present invention is a disazo compound represented by the following general formula (1):



In the general formula (1),  $R^{1A}$ ,  $R^{1B}$ ,  $R^{2A}$  and  $R^{2B}$  are each independently a halogen atom, an alkyl group, a methoxy group, an amino group, a nitro group, an acetyl amido group ( $-\text{NHCOC}_3$ ), a methyl ester group ( $-\text{COOC}_3$ ) or a primary amide group ( $-\text{CONH}_2$ ). It is preferable that  $R^{1A}$ ,  $R^{1B}$ ,  $R^{2A}$  and  $R^{2B}$  are each independently a methyl group, a methoxy group, an amino group, a nitro group, an acetyl amido group or a primary amide group. It is more preferable that  $R^{1A}$  and  $R^{2B}$  are methyl groups, and  $R^{1B}$  and  $R^{2A}$  are primary amide groups. Each of  $R^{1A}$ ,  $R^{1B}$ ,  $R^{2A}$  and  $R^{2B}$  may have a bond with any carbon atom on the benzene ring (except the carbon atom bound to the azo group ( $-\text{N}=\text{N}-$ )).

In the general formula (1),  $a1$  and  $b1$  are positive integers that a sum of the positive integers is 1 or more and 3 or less, and  $a2$  and  $b2$  are positive integers that a sum of the positive integers is 1 or more and 3 or less. It is preferable that  $a1$ ,  $b1$ ,  $a2$  and  $b2$  are each 1.

In the general formula (1),  $R^3$  is a halogen atom and is preferably a chlorine atom.  $R^3$  may have a bond with any carbon atom on the benzene ring (except the carbon atoms bound to the amide groups ( $-\text{CO}-\text{NH}-$ )).

In the general formula (1),  $c$  is an integer of 1 or more and 3 or less, and it is preferably 1.

In the general formula (1),  $R^4$  and  $R^5$  are each independently a halogen atom, an alkyl group, a methoxy group, an amino group, a nitro group, an acetyl amido group ( $-\text{NHCOC}_3$ ), an acetyl group ( $-\text{COCH}_3$ ), a methyl ester group ( $-\text{COOC}_3$ ) or a primary amide group ( $-\text{CONH}_2$ ). It is preferable that  $R^4$  and  $R^5$  are acetyl groups.

In the general formula (1),  $d$  and  $e$  are each independently 1 or 2. It is preferable that  $d$  and  $e$  are 1.

As the compound A represented by the general formula (1), examples include, but are not limited to, the following compounds. Of the following examples, the compound represented by the following formula (1A) is C.I. Pigment Yellow 214 (CAS No. 254430-12-5) and the compound represented by the following formula (1B) is C.I. Pigment Yellow 219 (CAS No. 347174-87-2).

The compound A used in the present invention is not limited to the following examples. Tautomers of the following examples can be also preferably used as the compound A of the present invention.



The compound A may be a commercially-available product or may be synthesized in advance.

As the method for synthesizing the compound A, examples include, but are not limited to, a method of coupling one equivalent of an N,N'-1,4-diacetylphenylene-diamine derivative represented by the following general formula (a) with two equivalents of a benzenediazonium derivative represented by the following general formula (b) (see Japanese Examined Patent Application Publication No. 48-13692).



where R<sup>3</sup>, R<sup>4</sup> and R<sup>5</sup> are the same groups as R<sup>3</sup>, R<sup>4</sup> and R<sup>5</sup> in the general formula (1), respectively, and c, d and e are the same numbers as c, d and e in the general formula (1), respectively.



where R<sup>1A'</sup> is the same group as R<sup>1A</sup> or R<sup>2A</sup> in the general formula (1); R<sup>1B'</sup> is the same group as R<sup>1B</sup> or R<sup>2B</sup> in the general formula (1); a1' is the same number as a1 or a2 in the general formula (1); and b1' is the same number as b1 or b2 in the general formula (1).

In the present invention, besides the compound A, the compound B represented by the following general formula (2) is contained as the yellow colorant.



In the general formula (2), the alkyl group as R<sup>6</sup> preferably has 5 to 30 carbon atoms, more preferably 10 to 25 carbon atoms, and still more preferably 15 to 20 carbon atoms.

As the compound B, examples include, but not limited to, C.I. solvent yellow 98 (CAS No. 12671-74-8, R<sup>6</sup>—(CH<sub>2</sub>)<sub>17</sub>(CH<sub>3</sub>).

With respect to 100 parts by mass of the binder resin, the total content of the compound A and the compound B is from 3 to 30 parts by mass, preferably from 4 to 25 parts by mass, more preferably from 6 to 20 parts by mass, and still more preferably from 8 to 18 parts by mass.

A traditional combination of yellow colorants has the following problem: when the compound A is used in an amount of more than 8 parts by mass with respect to 100 parts by mass of the binder resin, toner particles thus obtained vary in particle diameter and have poor particle size distribution. However, by using the compound A in combination with the compound B, poor particle size distribution is not obtained even if the compound A is used in an amount of more than 8 parts by mass, and toner particles with a target particle diameter can be obtained.

When the total content of the compound A and the compound B is less than 3 part by mass with respect to 100 parts by mass of the binder resin, a target chroma is not obtained. On the other hand, when the total content is more than 30 parts by mass, the effect exerted on chroma by the addition of the compounds A and B is saturated and economically disadvantageous.

In the present invention, the mass ratio of the content of the compound A to the content of the compound B (compound A/compound B) is from 0.8 to 20.

When the mass ratio is less than 0.8, the content of the compound B is too large and results in poor light resistance. This is because a dye like the compound B is liable to UV-induced color deterioration. On the other hand, when the mass ratio is more than 20, there is a decrease in chroma.

Since the mass ratio (compound A/compound B) is from 0.8 to 20, reflection density, chroma and light resistance can be increased with balance.

The content of the compound A is preferably from 1 to 28 parts by mass, more preferably from 3 to 20 parts by mass, and still more preferably from 5 to 15 parts by mass, with respect to 100 parts by mass of the binder resin. When the content of the compound A is less than 1 part by mass with respect to 100 parts by mass of the binder resin, a remarkable decrease in reflection density may occur. When the content of the compound A is more than 28 parts by mass with respect to 100 parts by mass of the binder resin, an increase in monomer viscosity may occur during the production process, and handling may be difficult.

The content of the compound B is preferably from 0.5 to 12 parts by mass, more preferably from 1 to 6 parts by mass, and still more preferably from 1.5 to 6 parts by mass, with respect to 100 parts by mass of the binder resin. When the

content of the compound B is less than 0.5 part by mass with respect to 100 parts by mass of the binder resin, a target chroma may not be obtained. When the content of the compound B is more than 12 parts by mass with respect to 100 parts by mass of the binder resin, poor light resistance may be obtained. This is because a dye like the compound B is liable to UV-induced color deterioration.

The principle of the effect provided by the use of the combination of the compounds A and B, is not clear. However, it is considered as follows: by using the combination of the compounds, the dispersion stability of the compounds in the polymerizable monomer composition or binder resin is increased; therefore, the yellow toner thus obtained is a toner which provides a sharper color than ever before and which has excellent light resistance. Also, by the use of the combination of the compounds A and B, the particle size distribution of the colored resin particles with a target particle diameter can be narrow.

As another additive, a positively or negatively chargeable charge control agent can be used to improve the chargeability of the toner.

The charge control agent is not particularly limited, as long as it is one that is generally used as a charge control agent for toners. Among charge control agents, a positively or negatively chargeable charge control resin is preferred, since the charge control resin is highly compatible with the polymerizable monomer and can impart stable chargeability (charge stability) to the toner particles. From the viewpoint of obtaining a positively chargeable toner, a positively chargeable charge control resin is more preferred.

As the positively chargeable charge control agent, examples include, but are not limited to, a nigrosine dye; a quaternary ammonium salt; a triaminotriphenylmethane compound; an imidazole compound; and a polyamine resin, a quaternary ammonium group-containing copolymer, and a quaternary ammonium salt group-containing copolymer, which are preferably used as the charge control resin.

As the negatively chargeable charge control agent, examples include, but are not limited to, an azo dye containing a metal such as Cr, Co, Al and Fe; a metal salicylate compound; a metal alkylsalicylate compound; and a sulfonic acid group-containing copolymer, a sulfonic acid salt group-containing copolymer, a carboxylic acid group-containing copolymer and a carboxylic acid salt group-containing copolymer, which are preferably used as the charge control resin.

In the present invention, it is desirable that the amount of the charge control agent is generally from 0.01 to 10 parts by mass, and preferably from 0.03 to 8 parts by mass, with respect to 100 parts by mass of the monovinyl monomer. When the added amount of the charge control agent is less than 0.01 part by mass, fog may occur. On the other hand, when the added amount of the charge control agent is more than 10 parts by mass, soiling in printing may occur.

As another additive, a molecular weight modifier is preferably used in the polymerization of the polymerizable monomer that is polymerized into a binder resin.

The molecular weight modifier is not particularly limited, as long as it is one that is generally used as a molecular weight modifier for toners. As the molecular weight modifier, examples include, but are not limited to, mercaptans such as t-dodecyl mercaptan, n-dodecyl mercaptan, n-octyl mercaptan and 2,2,4,6,6-pentamethylheptane-4-thiol, and thiuram disulfides such as tetramethyl thiuram disulfide, tetraethyl thiuram disulfide, tetrabutyl thiuram disulfide, N,N'-dimethyl-N,N'-diphenyl thiuram disulfide, and N,N'-dioctadecyl-N,N'-diisopropyl thiuram disulfide. These

molecular weight modifiers may be used alone or in combination of two or more kinds.

In the present invention, it is desirable that the amount of the molecular weight modifier is generally from 0.01 to 10 parts by mass, and preferably 0.1 to 5 parts by mass, with respect to 100 parts by mass of the monovinyl monomer.

As another additive, it is preferable to add a release agent. By adding the release agent, the releasability of the toner from a fixing roller upon fixing, can be improved. The release agent is not particularly limited, as long as it is one that is generally used as a release agent in toner. As the release agent, examples include, but are not limited to, low-molecular-weight polyolefin waxes and modified waxes thereof; natural plant waxes such as jojoba; petroleum waxes such as paraffin; mineral waxes such as ozokerite; synthetic waxes such as Fischer-Tropsch wax; and polyalcohol esters such as dipentaerythritol ester. Of them, polyalcohol esters are preferred since the toner can achieve a balance between storage stability and low-temperature fixability. These release agents may be used alone or in combination of two or more kinds.

The amount of the release agent is preferably from 0.1 to 30 parts by mass, and more preferably from 1 to 20 parts by mass, with respect to 100 parts by mass of the monovinyl monomer.

#### (A-2) Suspension Process of Obtaining Suspension (Droplets Forming Process)

In the present invention, the polymerizable monomer composition containing the polymerizable monomer and the yellow colorant is dispersed in an aqueous medium containing a dispersion stabilizer, and a polymerization initiator is added therein. Then, the polymerizable monomer composition are formed into droplets. The method for forming the droplets is not particularly limited. For example, the droplets are formed by means of a device capable of strong stirring, such as an (in-line type) emulsifying and dispersing machine (product name: Milder, manufactured by: Pacific Machinery & Engineering Co., Ltd.) and a high-speed emulsifying and dispersing machine (product name: T. K. Homomixer Mark II, manufactured by: PRIMIX Corporation).

As the polymerization initiator, examples include, but are not limited to, persulfates such as potassium persulfate and ammonium persulfate; azo compounds such as 4,4'-azobis (4-cyanovaleic acid), 2,2'-azobis(2-methyl-N-(2-hydroxyethyl)propionamide), 2,2'-azobis(2-amidinopropane)dihydrochloride, 2,2'-azobis(2,4-dimethylvaleronitrile) and 2,2'-azobisisobutyronitrile; and organic peroxides such as di-t-butylperoxide, benzoylperoxide, t-butylperoxy-2-ethylhexanoate, t-hexylperoxy-2-ethylbutanoate, diisopropylperoxydicarbonate, di-t-butylperoxyisophthalate and t-butylperoxyisobutyrate. They can be used alone or in combination of two or more kinds. Among them, organic peroxides are preferred since they can reduce residual polymerizable monomer and impart excellent printing durability.

Among organic peroxides, preferred are peroxy esters, and more preferred are non-aromatic peroxy esters, i.e., peroxy esters having no aromatic ring, since they have excellent initiator efficiency and can reduce residual polymerizable monomer.

The polymerization initiator may be added after the polymerizable monomer composition is dispersed into the aqueous medium and before the polymerizable monomer composition is formed into droplets as described above, or it may be added to the polymerizable monomer composition before the polymerizable monomer composition is dispersed into the aqueous medium.

## 11

The added amount of the polymerization initiator used for the polymerization of the polymerizable monomer composition, is preferably from 0.1 to 20 parts by mass, more preferably from 0.3 to 15 parts by mass, and even more preferably from 1 to 10 parts by mass, with respect to 100 parts by mass of the monovinyl monomer.

In the present invention, the aqueous medium means a medium containing water as a main component.

In the present invention, the dispersion stabilizer is preferably added to the aqueous medium. As the dispersion stabilizer, examples include, but are not limited to, inorganic compounds including sulfates such as barium sulfate and calcium sulfate, carbonates such as barium carbonate, calcium carbonate and magnesium carbonate, phosphates such as calcium phosphate, metal oxides such as aluminum oxide and titanium oxide, and metal hydroxides such as aluminum hydroxide, magnesium hydroxide and iron (II) hydroxide, and organic compounds including water-soluble polymers such as polyvinyl alcohol, methyl cellulose and gelatin, anionic surfactants, nonionic surfactants, and ampholytic surfactants. These dispersion stabilizers can be used alone or in combination of two or more kinds.

Among the above dispersion stabilizers, preferred are colloids of inorganic compounds, and particularly preferred is a colloid of a hardly water-soluble metal hydroxide. By using a colloid of an inorganic compound, particularly a colloid of a hardly water-soluble metal hydroxide, the colored resin particles can have a narrow particle size distribution, and the amount of the dispersion stabilizer remaining after washing can be small, so that the polymerization toner thus obtained can clearly reproduce an image and does not deteriorate environmental stability.

## (A-3) Polymerization Process

Formation of the droplets is carried out as described under the above (A-2). The thus-obtained aqueous dispersion medium is heated to polymerize, thereby forming an aqueous dispersion containing the yellow colorant.

The polymerization temperature of the polymerizable monomer composition is preferably 50° C. or more, and more preferably from 60 to 95° C. The polymerization reaction time is preferably from 1 to 20 hours, and more preferably from 2 to 15 hours.

The colored resin particles may be used as they are as a polymerization toner, or they may be mixed with an external additive and used as a polymerization toner. It is preferable that the colored resin particles are so-called core-shell type (or "capsule type") colored resin particles obtained by using the colored resin particles as a core layer and forming a shell layer, which is a layer that is different from the core layer, around the core layer. By covering the core layer composed of a substance having a low softening point with a substance having a higher softening point, the core-shell type colored resin particles can achieve a balance between lowering of fixing temperature and prevention of aggregation during storage.

A method for producing the above-mentioned core-shell type colored resin particles using the colored resin particles, is not particularly limited. The core-shell type colored resin particles can be produced by a conventional method. The in situ polymerization method and the phase separation method are preferable from the viewpoint of production efficiency.

Hereinafter, the method for producing the core-shell type colored resin particles by the in situ polymerization method, will be described.

The core-shell type colored resin particles can be obtained by adding a polymerizable monomer for forming a shell layer (a polymerizable monomer for shell) and a polymer-

## 12

ization initiator to an aqueous medium in which the colored resin particles are dispersed, and then polymerizing the mixture.

As the polymerizable monomer for shell, the above-mentioned polymerizable monomers can be used. Among the polymerizable monomers, it is preferable to use monomers that can provide a polymer having a Tg of more than 8° C., such as styrene, acrylonitrile and methyl methacrylate, alone or in combination of two or more kinds.

As the polymerization initiator used for polymerization of the polymerizable monomer for shell, examples include, but are not limited to, water-soluble polymerization initiators including metal persulfates such as potassium persulfate, and ammonium persulfate, and azo-type initiators such as 2,2'-azobis(2-methyl-N-(2-hydroxyethyl)propionamide) and 2,2'-azobis(2-methyl-N-(1,1-bis(hydroxymethyl)2-hydroxyethyl)propionamide). These polymerization initiators can be used alone or in combination of two or more kinds. The amount of the polymerization initiator is preferably from 0.1 to 30 parts by mass, and more preferably from 1 to 20 parts by mass, with respect to 100 parts by mass of the polymerizable monomer for shell.

The polymerization temperature of the shell layer is preferably 50° C. or more, and more preferably from 60 to 95° C. The polymerization reaction time is preferably from 1 to 20 hours, and more preferably from 2 to 15 hours.

## (A-4) Washing, Filtering, Dehydrating and Drying Processes

After the polymerization is completed, the aqueous dispersion of the colored resin particles obtained by the polymerization is preferably subjected to operations of filtering, washing for removal of the dispersion stabilizer, dehydrating and drying, several times as needed, according to a conventional method.

The washing is preferably carried out by the following method. When the inorganic compound is used as the dispersion stabilizer, acid or alkali is added to the aqueous dispersion of the colored resin particles, thereby dissolving the dispersion stabilizer in water and removing it. When the colloid of the hardly water-soluble inorganic hydroxide is used as the dispersion stabilizer, the pH of the aqueous dispersion of the colored resin particles is controlled to 6.5 or less by adding acid. As the acid, examples include, but are not limited to, inorganic acids such as sulfuric acid, hydrochloric acid and nitric acid, and organic acids such as formic acid and acetic acid. Sulfuric acid is particularly preferred for its high removal efficiency and small impact on production facilities.

The dehydrating and filtering method is not particularly limited and can be selected from various known methods. As the method, examples include, but are not limited to, a centrifugal filtration method, a vacuum filtration method and a pressure filtration method. Also, the drying method is not particularly limited and can be selected from various methods.

## (B) Pulverization Method

In the case of producing the colored resin particles by employing the pulverization method, the colored resin particles are produced by the following processes.

First, a binder resin, a yellow colorant, and other additives added as needed, such as a charge control agent and a release agent, are mixed by means of a mixer such as a ball mill, a V-type mixer, FM Mixer (product name), a high-speed dissolver, an internal mixer or Forberg.

Next, while heating the thus-obtained mixture, the mixture is kneaded by means of a press kneader, a twin screw kneading machine, a roller or the like. The thus-obtained kneaded product is coarsely pulverized by means of a

pulverizer such as a hammer mill, a cutter mill or a roller mill, finely pulverized by means of a pulverizer such as a jet mill or a high-speed rotary pulverizer, and then classified into a desired particle diameter by means of a classifier such as a wind classifier or an airflow classifier, thereby obtaining the colored resin particles produced by the pulverization method.

In the pulverization method, those that are provided above under "(A) Suspension polymerization method" can be used as the binder resin, the yellow colorant, and the other additives added as needed, such as the charge control agent and the release agent. Similarly to the colored resin particles obtained by the above "(A) Suspension polymerization method", the colored resin particles obtained by the pulverization method can be core-shell type colored resin particles by a method such as the in situ polymerization method.

As the binder resin, resins that have been widely used for toners can be used. As the binder resin used in the pulverization method, examples include, but are not limited to, polystyrene, styrene-butyl acrylate copolymers, polyester resins and epoxy resins.

## 2. Colored Resin Particles

The colored resin particles containing the yellow colorant are obtained by the production method such as the above-mentioned "(A) Suspension polymerization method" or "(B) Pulverization method".

Hereinafter, the colored resin particles constituting the toner will be described. The colored resin particles described below encompass both core-shell type colored resin particles and colored resin particles of other types.

The volume average particle diameter (D<sub>v</sub>) of the colored resin particles is preferably from 3 to 15  $\mu\text{m}$ , and more preferably from 4 to 12  $\mu\text{m}$ . When the volume average particle diameter (D<sub>v</sub>) is less than 3  $\mu\text{m}$ , the flowability of the polymerization toner decreases and may deteriorate transferability or decrease image density. When the volume average particle diameter (D<sub>v</sub>) is more than 15  $\mu\text{m}$ , image resolution may decrease.

For the colored resin particles, the ratio (D<sub>v</sub>/D<sub>n</sub>) of the volume average particle diameter (D<sub>v</sub>) and the number-average particle diameter (D<sub>n</sub>) is preferably from 1.0 to 1.25, and more preferably from 1.0 to 1.2. When the ratio D<sub>v</sub>/D<sub>n</sub> is more than 1.3, there may be a decrease in transferability, image density and resolution. The volume average particle diameter and number average particle diameter of the colored resin particles can be measured by means of a particle size analyzer (product name: Multisizer, manufactured by: Beckman Coulter, Inc.), for example.

The average circularity of the colored resin particles of the present invention is preferably from 0.96 to 1.00, more preferably from 0.97 to 1.00, and even more preferably from 0.98 to 1.00, from the viewpoint of image reproducibility.

When the average circularity of the colored resin particles is less than 0.96, thin line reproducibility in printing may deteriorate.

As the toner of the present invention, the colored resin particles containing the yellow colorant can be used as they are. From the viewpoint of controlling the chargeability, flowability and storage stability of the toner, the colored resin particles may be used as a one-component toner by mixing and stirring the colored resin particles with the external additives to attach the external additives to the surface of the colored resin particles.

The one-component toner may be mixed and stirred with carrier particles to obtain a two-component developer.

A stirrer is used to cover the colored resin particles with the external additives. The stirrer is not particularly limited,

as long as it is a stirring device that can attach the external additives to the surface of the colored resin particles. For example, the colored resin particles can be covered with the external additives by means of a stirrer that is capable of mixing and stirring, such as FM Mixer (product name, manufactured by: Nippon Coke & Engineering Co., Ltd.), Super Mixer (product name, manufactured by: Kawata Manufacturing Co., Ltd.), Q Mixer (product name, manufactured by: Nippon Coke & Engineering Co., Ltd.), Mechanofusion System (product name, manufactured by: Hosokawa Micron Corporation) and Mechanomill (product name, manufactured by: Okada Seiko Co., Ltd.)

As the external additives, examples include, but are not limited to, inorganic fine particles composed of silica, titanium oxide, aluminum oxide, zinc oxide, tin oxide, calcium carbonate, calcium phosphate and/or cerium, oxide, and organic fine particles composed of polymethyl methacrylate resin, silicone resin and/or melamine resin. Of them, inorganic fine particles are preferred. Of inorganic fine particles, silica and/or titanium oxide is preferred, and fine particles composed of silica are particularly preferred.

These external additives can be used alone. However, it is preferable to use them in combination of two or more kinds.

In the present invention, it is desirable that the external additives are used in an amount of generally from 0.05 to 6 parts by mass, and preferably from 0.2 to 5 parts by mass, with respect to 100 parts by mass of the colored resin particles. When the added amount of the external additives is less than 0.05 part by mass, the toner may not be fully transferred and may partly remain on a roller. When the added amount of the external additives is more than 6 parts by mass, fog may occur.

## 4. Toner of the Present Invention

The toner of the present invention obtained through the above steps uses the combination of the compound A and the compound B as the yellow colorant: therefore, the toner of the present invention is a yellow toner which provides a sharper color than ever before in small amounts and which has excellent light resistance.

The light resistance of the toner of the present invention can be evaluated by the following method, for example.

(A) A commercially-available, non-magnetic one-component development color printer (printing rate: 20 sheets/min) was used. The toner cartridge of the development device is filled with a sample yellow toner, and printing sheets are loaded in the printer. Then, the printer is left to stand under an (N/N) environment at a temperature of 23° C. and a relative humidity of 50% for one day. Then, while the amount of the toner supplied onto the developing roller in solid pattern printing is fixed at 0.3 mg/cm<sup>2</sup>, sheets are continuously printed at an image density of 5%. Solid pattern printing (image density: 100%) is carried out on the tenth sheet. Using a McBeth transmitting image densitometer, the reflection density (image density) of the tenth sheet is measured.

(B) The reflection density (image density) is measured in the same condition as the above (A), except that the time to leave the printer to stand is 560 hours.

(C) A reflection density decrease rate is obtained by the following formula, using a value (ID<sub>ON</sub>) of the reflection density (image density) obtained in the above (A) and a value (ID<sub>560</sub>) of the reflection density (image density) obtained in the above (B).

$$\text{(Reflection density decrease rate)} = \frac{(ID_{ON} - ID_{560})}{ID_{ON}} \times 100(\%)$$

From the reflection density decrease rate thus obtained, the light resistance of the toner is evaluated in accordance with the following evaluation criteria. It is considered that as the reflection density decrease rate decreases, the toner can be left to stand for a long period of time and maintain the reflection density. Therefore, the toner can be evaluated as having excellent light resistance.

- o: The reflection density decrease rate is less than 8%.  
x: The reflection density decrease rate is 8% or more.

## EXAMPLES

Hereinafter, the present invention will be described further in detail, with reference to examples and comparative examples. However, the scope of the present invention may not be limited to the following examples. Herein, "part(s)" and "%" are based on mass if not particularly mentioned.

## 1. Production of Colored Resin Particles

## &lt;Colored Resin Particles (1)&gt;

## 1-1. Preparation of Polymerizable Monomer Composition for Core

The following raw materials were subjected to wet pulverization by means of a media-type disperser (product name: PICO MILL, manufactured by: Asada Iron Works Co., Ltd.): 75 parts of styrene, 25 parts of n-butyl acrylate, 0.1 part of a polymethacrylic acid ester macromonomer (product name: AA6, manufactured by: TOAGOSEI Co., Ltd., Tg: 94° C.), 0.7 part of divinylbenzene, 1.0 part of tetraethylthiuram disulfide and, as yellow colorant, 6 parts of C.I. Pigment Yellow 214 (represented by the following formula (1A), product name: PV Fast Yellow H9G VP2430, manufactured by: Clariant Corp., CAS No. 254430-12-5) and 4 parts of C.I. Solvent Yellow 98 (product name: Hostasol Yellow 3G, manufactured by: Clariant Corp., CAS No. 12671-74-8). To a mixture obtained by the wet pulverization, 1.2 parts of a charge control resin (product name: Acrybase FCA-161P, manufactured by: Fujikura Kasei Co., Ltd.) and 10 parts of an ester wax (product name: WEP7, manufactured by: NOF Corporation) were added, mixed and dissolved to obtain a polymerizable monomer composition.



## 1-2. Preparation of Aqueous Dispersion Medium

An aqueous solution of 7.3 parts of sodium hydroxide dissolved in 50 parts of ion-exchanged water, was gradually added to an aqueous solution of 10.4 parts of magnesium chloride dissolved in 280 parts of ion-exchanged water, while stirring, thereby preparing a magnesium hydroxide colloid dispersion.

## 1-3. Preparation of Polymerizable Monomer for Shell

Meanwhile, 2 parts of methyl methacrylate and 130 parts of water were subjected to a fine dispersion treatment by means of an ultrasonic emulsifying machine, thereby preparing an aqueous dispersion of a polymerizable monomer for shell.

## 1-4. Droplets Forming Process

The polymerizable monomer composition was put in the magnesium hydroxide colloid dispersion (the magnesium hydroxide colloid amount: 5.3 parts) and stirred. Then, as a polymerization initiator, 6 parts of t-butylperoxy-2-ethylhexanoate was added thereto. The dispersion containing the polymerization initiator was subjected to dispersion at 15,000 rpm using an in-line type emulsifying and dispersing machine (product name: Milder, manufactured by: Pacific Machinery & Engineering Co., Ltd.), thereby forming the polymerizable monomer composition into droplets.

## 1-5. Suspension Polymerization Process

The dispersion containing the droplets of the polymerizable monomer composition was put in a reactor. The temperature thereof was increased to 90° C. to start a polymerization reaction. After the polymerization conversion rate reached almost 100%, a solution obtained by dissolving 0.1 part of 2,2'-azobis[2-methyl-N-(2-hydroxyethyl)-propionamide] (a water-soluble polymerization initiator, product name: VA-086, manufactured by: Wako Pure Chemical Industries, Ltd.) in the aqueous dispersion for the polymerizable monomer for shell, was added in the reactor. Next, the temperature of the reactor was kept at 95° C. for 4 hours to continue the polymerization further. Then, the reactor was cooled by water to stop the reaction, thereby obtaining an aqueous dispersion of core-shell type colored resin particles.

## 1-6. Post-Treatment Process

The aqueous dispersion of the colored resin particles was subjected to acid washing (25° C., 10 minutes) in which, while stirring the aqueous dispersion, sulfuric acid was added thereto until the pH of the aqueous dispersion was 4.5 or less. Then, the colored resin particles were separated from the aqueous dispersion by filtration and washed with water. The washing water was filtered. A filtrate thus obtained had an electrical conductivity of 20 µS/cm. The colored resin particles subjected to the washing and filtering processes were dehydrated and dried to obtain dried colored resin particles (1).

## &lt;Colored Resin Particles (2)&gt;

Colored resin particles (2) were obtained in the same manner as the production method of the colored resin particles (1), except that in the "Preparation of polymerizable monomer composition for core", the added amount of C.I. Pigment Yellow 214 was changed from 6 parts to 10 parts, and the added amount of C.I. Solvent Yellow 98 was changed from 4 parts to 2 parts.

## &lt;Colored Resin Particles (3)&gt;

Colored resin particles (3) were obtained in the same manner as the production method of the colored resin particles (1), except that in the "Preparation of polymerizable monomer composition for core", the added amount of C.I. Pigment Yellow 214 was changed from 6 parts to 10 parts.

## &lt;Colored Resin Particles (4)&gt;

Colored resin particles (4) were obtained in the same manner as the production method of the colored resin particles (1), except that in the "Preparation of polymerizable monomer composition for core", 4 parts of C.I. Solvent Yellow 98 was changed to 4 parts of C.I. Solvent Yellow 162 (represented by the following formula (X), product name: NEPTUN YELLOW 075, manufactured by: BASF, CAS No. 104244-10-2).



Formula (X)

## &lt;Colored Resin Particles (5)&gt;

Colored resin particles (5) were obtained in the same manner as the production method of the colored resin particles (1), except that in the “Preparation of polymerizable monomer composition for core”, 4 parts of C.I. Solvent Yellow 98 was changed to 4 parts of C.I. Solvent Yellow 93 (represented by the following formula (Y), product name: Solvaperm Yellow 3G, manufactured by: Clariant Corp., CAS No. 4702-90-3).



Formula (Y)

## &lt;Colored Resin Particles (6)&gt;

Colored resin particles (6) were obtained in the same manner as the production method of the colored resin particles (1), except that in the “Preparation of polymerizable monomer composition for core”, 4 parts of C.I. Solvent Yellow 98 was changed to 4 parts of C.I. Solvent Yellow 114 (represented by the following formula (Z), product name: Solvaperm Yellow 2G, manufactured by: Clariant Corp., CAS No. 7576-65-0).



Formula (Z)

## &lt;Colored Resin Particles (7)&gt;

Colored resin particles (7) were obtained in the same manner as the production method of the colored resin particles (1), except that in the “Preparation of polymerizable monomer composition for core”, the added amount of C.I. Pigment Yellow 214 was changed from 6 parts to 8 parts, and 4 parts of C.I. Solvent Yellow 98 was not used.

2. Evaluation of Properties of Colored Resin Particles

Measurement of volume average particle diameter (D<sub>v</sub>) and calculation of particle size distribution (D<sub>v</sub>/D<sub>n</sub>) were carried out on the colored resin particles (1) to (7).

First, 0.1 g of a measurement sample (colored resin particles) was weighed, out and put in a beaker. As a dispersant, 0.1 mL of an alkylbenzene sulfonic acid aqueous solution (product name: Driwel, manufactured by: Fujifilm Corporation) was added thereto. In addition, 10 to 30 mL of Isoton II was added to the beaker. The mixture was dispersed for three minutes with a 20 W ultrasonic disperser. Then, the volume average particle diameter (D<sub>v</sub>) and number average particle diameter (D<sub>n</sub>) of the colored resin particles were measured with a particle diameter measuring device (product name: Multisizer, manufactured by: Beckman Coulter, Inc.) in the following conditions:

Aperture diameter: 100  $\mu$ m

Medium: Isoton II

Number of measured particles: 100,000

Next, the particle size distribution (D<sub>v</sub>/D<sub>n</sub>) of the colored resin particles was calculated.

## 3. Production of Yellow Toner

The colored resin particles (1) to (7) were covered with external additives to produce yellow toners of Examples 1 to 3 and Comparative Examples 1 to 4.

## Example 1

First, 0.6 part of hydrophobized silica fine particles having an average particle diameter of 7 nm and 1 part of hydrophobized silica fine particles having an average particle diameter of 35 nm, were added to 100 parts of the colored resin particles (1). They were mixed by means of a high-speed stirrer (product name: FM Mixer, manufactured by: Nippon Coke & Engineering Co., Ltd.) to prepare the yellow toner of Example 1.

## Examples 2 and 3 and Comparative Examples 1 to 4

The yellow toners of Examples 2 and 3 and Comparative Examples 1 to 4 were obtained in the same manner as Example 1, except that the colored resin particles (1) were changed to, as shown in the following Table 1, any of the colored resin particles (2) to (7).

## 4. Evaluation of Toners for Developing Electrostatic Images

The charge amount, reflection density (image density), luminance (L\*), color coordinate (a\*, b\*) and chroma (C\*) of the yellow toners of Examples 1 to 3 and Comparative Examples 1 to 4, were measured as follows. Also, the light resistance of the yellow toners was evaluated as follows.

## 4-1. Measurement of Charge Amount

The toner cartridge of a commercially-available, non-magnetic one-component development printer (product name: MFC-9840-CDW, manufactured by: Brother Industries, Ltd.) was filled with a sample yellow toner, and printing sheets were loaded in the printer. Then, the printer was left to stand under an environment at a temperature of 23° C. and a humidity of 50% (NN environment) for one day. Then, under the same NN environment, solid pattern printing (image density: 0%) was carried out on one sheet. When printing halfway, the printer was stopped. The toner supported on the developing roller was suctioned using a suction type Q/m analyzer (product name: 210HS-2A, manufactured by: TREK JAPAN) to measure the charge amount of the toner. The measured charge amount was converted, into the charge amount Q/M ( $\mu$ C/g) per unit mass of the toner.

4-2. Measurement of Reflection Density, Luminance, Color Coordinate and Chroma

A commercially-available, non-magnetic one-component development color printer (printing rate: 20 sheets/min) was used. The toner cartridge of the development device was filled with a sample yellow toner, and printing sheets were loaded in the printer. Then, the printer was left to stand under an (N/N) environment at a temperature of 23° C. and a relative humidity of 50% for one day. Then, while the amount of the toner supplied onto the developing roller in solid pattern printing was fixed at 0.3 mg/cm<sup>2</sup>, sheets were continuously printed at an image density of 5%. Solid pattern printing (image density: 100%) was carried out on the tenth sheet. Using a McBeth transmitting image densitometer, the reflection density (image density), luminance (L\*), color coordinate (a\*, b\*) and chroma (C\*) of the tenth sheet were measured.

4-3. Evaluation of Light Resistance

The light resistance of the toner was evaluated based on a reflection density decrease rate obtained from the value of the reflection density obtained in the above “4-2. Measurement of reflection density, luminance, color coordinate and chroma” and the value of the reflection density obtained after the printer was left to stand for a long period of time (560 hours).

The same color printer as above was used. The toner cartridge of the development device was filled with a sample yellow toner, and printing sheets were loaded in the printer. Then, the printer was left to stand under an (N/N) environment at a temperature of 23° C. and a relative humidity of

50% for 560 hours. Then, in the same condition, sheets were continuously printed, and solid pattern printing (image density: 100%) was carried out on the tenth sheet. Using a McBeth transmitting image densitometer, the reflection density (image density) of the tenth sheet was measured. A reflection density decrease rate was obtained by the following formula, using, as just described, the value (ID<sub>560</sub>) of the reflection density (image density) obtained after the printer was left to stand for 560 hours, and the value (ID<sub>ON</sub>) of the reflection density (image density) obtained in the above “4-2. Measurement of reflection density, luminance, color coordinate and chroma”.

$$(1) \text{Reflection density decrease rate} = \frac{(ID_{ON} - ID_{560})}{ID_{ON}} \times 100\%$$

From the reflection density decrease rate thus obtained, the light resistance of the toner was evaluated in accordance with the following evaluation criteria.

o: The reflection density decrease rate is less than 8%.

x: The reflection density decrease rate is 8% or more.

Table 1 shows the measurement and evaluation results of the yellow toners of Examples 1 to 3 and Comparative Examples 1 to 4, along with the toner composition.

In the following Table 1, “PY2.14” means C.I. Pigment Yellow 214; “SY98” means C.I. Solvent Yellow 98; “SY162” means C.I. Solvent Yellow 162; “SY93” means C.I. Solvent Yellow 93; and “SY114” means C.I. Solvent Yellow 114. Also, “Compound A+compound B (parts)” means the sum of the added amount of the compound A and that of the compound B.

TABLE 1

|                                                | Example 1     | Example 2     | Example 3     | Comparative Example 1 | Comparative Example 2 | Comparative Example 3 | Comparative Example 4 |
|------------------------------------------------|---------------|---------------|---------------|-----------------------|-----------------------|-----------------------|-----------------------|
| Colored resin particles                        | Particles (1) | Particles (2) | Particles (3) | Particles (4)         | Particles (5)         | Particles (6)         | Particles (7)         |
| Compound A                                     | PY214         | PY214         | PY214         | PY214                 | PY214                 | PY214                 | PY214                 |
| Added amount (parts)                           | 6             | 10            | 10            | 6                     | 6                     | 6                     | 8                     |
| Compound B                                     | SY98          | SY98          | SY98          | —                     | —                     | —                     | —                     |
| Added amount (arts)                            | 4             | 2             | 4             | —                     | —                     | —                     | —                     |
| Compound A + compound B (parts)                | 10            | 12            | 14            | 6                     | 6                     | 6                     | 8                     |
| Ratio of compound A/compound B                 | 1.5           | 5.0           | 2.5           | —                     | —                     | —                     | —                     |
| Other yellow pigment                           | —             | —             | —             | SY162                 | SY93                  | SY114                 | —                     |
| Added amount (parts)                           | —             | —             | —             | 4                     | 4                     | 4                     | —                     |
| D <sub>v</sub> (μm)                            | 6.0           | 5.4           | 5.5           | 5.8                   | 5.9                   | 11.1                  | 12.9                  |
| D <sub>v</sub> /D <sub>n</sub>                 | 1.19          | 1.23          | 1.21          | 1.17                  | 1.28                  | 2.34                  | 1.37                  |
| Charge amount (μC/g)                           | 28            | 25            | 34            | 26                    | -8                    | 13                    | 15                    |
| Printing evaluation                            |               |               |               |                       |                       |                       |                       |
| Amount of toner on sheet (mg/cm <sup>2</sup> ) | 0.3           | 0.3           | 0.3           | 0.3                   | 0.3                   | 0.3                   | 0.3                   |
| Reflection density                             | 1.15          | 1.10          | 1.17          | 1.38                  | —                     | 1.24                  | 1.05                  |
| Luminance L*                                   | 94.7          | 98.7          | 93.2          | 95.4                  | —                     | 94.3                  | 95.4                  |
| a*                                             | -6.5          | -11.7         | -7.5          | -11.9                 | —                     | -8.7                  | -10.9                 |
| b*                                             | 90.6          | 88.7          | 89.7          | 87.5                  | —                     | 81.5                  | 69.7                  |
| Chroma C*                                      | 90.8          | 89.5          | 90.0          | 88.3                  | —                     | 81.9                  | 70.5                  |
| Hue angle (°)                                  | 94.1          | 97.5          | 94.6          | 97.8                  | —                     | 96.1                  | 98.9                  |

TABLE 1-continued

| Example 1                        | Example 2 | Example 3 | Comparative Example 1 | Comparative Example 2 | Comparative Example 3 | Comparative Example 4 |
|----------------------------------|-----------|-----------|-----------------------|-----------------------|-----------------------|-----------------------|
| Light resistance evaluation      |           |           |                       |                       |                       |                       |
| Reflection density decrease rate | ○         | ○         | ○                     | X                     | —                     | X                     |

## 5. Evaluation of Toners

The yellow toner of Comparative Example 1 is a toner using the compound A (C.I. Pigment Yellow 214) in combination with C.I. Solvent Yellow 162. For Comparative Example 1, the chroma C\* is as low as 88.3, and the light resistance evaluation result is "x". Therefore, it is clear that the yellow toner is dull in color and poor in light resistance when C.I. Solvent Yellow 162 is used in place of the compound B, and the toner on the sheet is 0.3 mg/cm<sup>2</sup> and smaller than ever before.

The yellow toner of Comparative Example 2 is a toner using the compound A (C.I. Pigment Yellow 214) in combination with C.I. Solvent Yellow 93. For Comparative Example 2, the charge amount is as low as -8 μC/g. Since the toner was negatively charged, toner particles with originally expected charging ability were not obtained, and a toner that was worthy of printing evaluation was not obtained. Therefore, printing evaluation of the toner was cancelled.

The yellow toner of Comparative Example 3 is a toner using the compound A (C.I. Pigment Yellow 214) in combination with C.I. Solvent Yellow 114. For Comparative Example 3, the volume average particle diameter (D<sub>v</sub>) is as large as 11.1 μm, and the particle size distribution (D<sub>v</sub>/D<sub>n</sub>) is 2.34. Accordingly, the yellow toner of Comparative Example 3 is a toner with a wide particle size distribution. Also, the light resistance evaluation result is "x". From these results, it is clear that when C.I. Solvent Yellow 114 is used in place of the compound B, the particle diameter of the toner thus obtained increases overall; the toner particles are non-uniform in particle diameter; and the toner thus obtained is poor in light resistance.

The yellow toner of Comparative Example 4 is a toner in which 8.0 parts by mass of the compound A is only used as the yellow colorant with respect to 100 parts by mass of the binder resin. For Comparative Example 4, the volume average particle diameter (D<sub>v</sub>) is as large as 12.9 μm, and the particle size distribution (D<sub>v</sub>/D<sub>n</sub>) is 1.37. Accordingly, the yellow toner of Comparative Example 3 is a toner with a wide particle size distribution. From these results, it is clear that when the compound B is not used, the particle diameter of the toner thus obtained increases overall, and the toner particles are non-uniform in particle diameter.

Also for Comparative Example 4, the chroma C\* is as low as 70.5. This value is the lowest among the evaluated toners. Therefore, it is clear that the yellow toner is especially dull in color when the compound A is used solely as the yellow colorant, and the toner on the sheet is 0.3 mg/cm<sup>2</sup> and smaller than ever before.

Meanwhile, the yellow toners of Examples 1 to 3 are toners in which the total content of the compound A and the compound B is from 10 to 14 parts by mass with respect to 100 parts by mass of the binder resin, and the mass ratio of the content of the compound A to the content of the compound B (compound A/compound B) is from 1.5 to 5.0.

For Examples 1 to 3, the volume average particle diameter (D<sub>v</sub>) is as small as 5.4 to 6.0 μm, and the particle size distribution (D<sub>v</sub>/D<sub>n</sub>) is as narrow as 1.19 to 1.23. Therefore, it is clear that the toners of Examples 1 to 3 have the desired particle diameter and are narrow in particle size distribution.

Also for Examples 1 to 3, the chroma C\* is as high as 89.5 or more, and the light resistance evaluation result is "o". Therefore, it is clear that even when the toner on the sheet is 0.3 mg/cm<sup>2</sup> and smaller than ever before, the yellow toners of Examples 1 to 3 (in which the total content of the compounds A and B contained as the yellow colorant is from 3 to 30 parts by mass with respect to 100 parts by mass of the binder resin, and the mass ratio of the content of the compound A to the content of the compound B (compound A/compound B) is from 0.8 to 20) are each a toner which provides a sharper color than ever before and which has excellent light resistance.

The invention claimed is:

1. A yellow toner comprising a binder resin and a yellow colorant,

wherein a compound A represented by the following general formula (1) and a compound B represented by the following general formula (2) are contained as the yellow colorant, and

wherein a total content of the compound A and the compound B is from 3 to 30 parts by mass with respect to 100 parts by mass of the binder resin, and a mass ratio of the content of the compound A to the content of the compound B (compound A/compound B) is from 0.8 to 20:

General Formula (1)



where R<sup>1A</sup>, R<sup>1B</sup>, R<sup>2A</sup> and R<sup>2B</sup> are each independently a halogen atom, an alkyl group, a methoxy group, an amino group, a nitro group, an acetyl amido group (—NHCOCH<sub>3</sub>), a methyl ester group (—COOCH<sub>3</sub>) or a primary amide group (—CONH<sub>2</sub>); R<sup>3</sup> is a halogen atom; R<sup>4</sup> and R<sup>5</sup> are each independently a halogen atom, an alkyl group, a methoxy group, an amino group, a nitro group, an acetyl amido group (—NHCOCH<sub>3</sub>), an acetyl group (—COCH<sub>3</sub>), a methyl ester group (—COOCH<sub>3</sub>) or a primary amide group (—CONH<sub>2</sub>); a<sub>1</sub> and b<sub>1</sub> are positive integers that a sum of the positive integers is 2 or 3; a<sub>2</sub> and b<sub>2</sub> are positive integers that a sum of the positive integers is 2 or 3; c is an integer of 1 or more and 3 or less; and d and e are each independently 1 or 2,

General Formula (2)



where  $R^6$  is an alkyl group.

2. The yellow toner according to claim 1, wherein the compound A represented by the general formula (1) is selected from the group consisting of C.I. Pigment Yellow 214 and C.I. Pigment Yellow 219.

3. The yellow toner according to claim 1, wherein the compound B represented by the general formula (2) is C.I. Solvent Yellow 98.

4. The yellow toner according to claim 1, wherein a content of the compound A is 1 to 28 parts by mass with respect to 100 parts by mass of the binder resin.

5. The yellow toner according to claim 1, wherein a content of the compound B is 0.5 to 12 parts by mass with respect to 100 parts by mass of the binder resin.

\* \* \* \* \*